

Dec. 17, 1929.

A. L. CLAPP

1,739,578

SHOE STIFFENER

Filed Sept. 12, 1923



Inventor:  
Albert L. Clapp.  
by  
Albert Brown Brooklyn May  
Attest,

## UNITED STATES PATENT OFFICE

ALBERT L. CLAPP, OF DANVERS, MASSACHUSETTS, ASSIGNOR TO BECKWITH MANUFACTURING COMPANY, OF BOSTON, MASSACHUSETTS, A CORPORATION OF MASSACHUSETTS

## SHOE STIFFENER

Application filed September 12, 1923. Serial No. 662,223.

Shoe stiffeners are commonly constructed of fibrous sheet material saturated with thermo-plastic material, that is, material which is hard at atmospheric and body temperatures but which may be softened by subjecting it to a moderate degree of heat. The shoe stiffener is heated when being formed into the shoe and thereafter being allowed to cool in proper shape, becomes stiff and rigid and so normally remains during the life of the shoe. The thermo-plastic material is frequently softened by the application of dry heat and it is often found that when shoes having incorporated therein stiffeners saturated with such material are exposed to the sun, as for example when on display in show windows, the relatively intense heat causes the material to soften sufficiently to permit the stiffeners partially to collapse, thus impairing both the appearance of the shoes and their salability.

The object of the present invention is to prevent the possibility of this deformation of the stiffeners, due to such exposure, without impairing their capability of being softened sufficiently to be readily worked and shaped when the shoe is being made, and for this purpose it is proposed to employ in connection with the usual thermo-plastic material other material which may be softened only by the application of moist heat thereto, such material, for example, as water soluble gums or stiffening agents such as animal or fish glue. It has been found impracticable to saturate the fibrous material with glue and also with the thermo-plastic material. The glue when used alone does not possess properties necessary for its successful use as stiffening material for the fibrous base, since it is easily cracked and pulverized and is not waterproof. It is found, however, that a combination of the two, i. e. glue and a thermo-plastic compound, may be successfully employed by coating one face of the fibrous base with a, say, 5% to 10% glue solution so that it coats and partially saturates the material but does not saturate it throughout, permitting it to dry, and thereafter immersing the fibrous material in melted thermo-plastic agent which saturates the fibrous base

from the opposite face throughout and covers the glue.

Referring to the accompanying drawing which conventionally illustrates, much enlarged, a piece of the finished material, the 55 felt sheet is indicated at 1, the coating of glue applied to one face thereof and penetrating more or less between the adjacent fibers of the felt at 2, and the thermo-plastic saturant permeating the felt at 3 and coating the glue 60 surface at 4.

It is found in practice that the portion of the material saturated and coated with the glue is sufficiently stiff to cause the shoe stiffener formed therefrom to retain its shape 65 even when subjected to dry heat sufficient to soften the thermo-plastic compound and to cause the stiffener, without the presence of the glue, to lose its shape. But by subjecting the stiffener so treated to the action of both 70 moisture and heat, the glue, together with the thermo-plastic material, is softened so that the stiffener is reduced to a limp or plastic condition where it can be successfully worked 75 and shaped to the last.

Instead of animal glue, dextrine, starch, or other water soluble gums may also be used, but animal or fish glue has been found preferable. The presence of the thermo-plastic material also renders the stiffener waterproof, which it would not be by the use of glue alone, but the glue coating is covered with the thermo-plastic material in the saturating process and so is sufficiently protected to render it waterproof without causing it to be entirely inaccessible to the moist heat treatment to which it is subjected preparatory for the forming operation about the last. Where the glue is used, Montan wax may be employed as the thermo-plastic saturant for a 80 felt such as produced on a paper machine. Montan wax ordinarily can not be used satisfactorily alone in the impregnation of a paper felt where glue is not used, since it becomes 85 so fluid, when heated sufficiently to soften it that it acts as a lubricant and permits the fibers of a felt, such as produced on a paper machine, to pull apart. The presence of the glue, however, holds the fibers together and retains the wax and so make it possible to 90 95 100

use this material alone as the thermo-plastic saturant.

By the treatment herein outlined, it is seen that two stiffening agents of different characteristics, one being softenable by dry heat and the other requiring moisture in addition to heat, are employed in different portions of the thickness of the fibrous sheet material, each responding to heat treatment in its own way without modification by the other. One of these stiffening agents, as heretofore described, may be incorporated while in an aqueous vehicle, the water then being dried out and this agent allowed to harden. The other agent may then be incorporated when in melted condition. In the completed article the stiffness imparted by each agent is reducible under its own particular conditions of softening independently of the other so that the stiffener must be subjected to the conditions which will soften all the stiffening agents used in order to render it limp.

I claim:

- 25 1. A shoe stiffener comprising fibrous sheet material having one portion treated with a water soluble stiffening agent only and another portion with thermo-plastic material only.
- 30 2. A shoe stiffener comprising fibrous sheet material partially stiffened by a water soluble stiffening agent applied to one side and adapted to be softened by moist heat and saturated with thermo-plastic material.
- 35 3. A shoe stiffener comprising fibrous material stiffened by a water soluble stiffening agent and a thermoplastic agent, one of said agents enveloping the other.
- 40 4. A shoe stiffener comprising fibrous material having one portion saturated with a water soluble stiffening agent only and another portion saturated with a thermoplastic agent only.
- 45 5. A shoe stiffener comprising fibrous sheet material having a portion treated with a water soluble stiffening agent, and thermo-plastic material enveloping said treated portion and saturating the remainder of said material.
- 50 6. A shoe stiffener comprising fibrous sheet material, a water soluble stiffening agent applied to one face of said sheet material, and a thermoplastic enveloping said water soluble agent and with which said fibrous material is saturated.
- 55 7. A shoe stiffener comprising fibrous sheet material partially stiffened by a water soluble material and saturated with thermo-plastic material.
- 60 8. A shoe stiffener comprising fibrous sheet material coated on one face with glue, and saturated with Montan wax.
- 65 9. A shoe stiffener comprising fibrous sheet material coated on one face with glue, and

saturated with Montan wax, the wax also coating the glued face.

10. A shoe stiffener comprising fibrous sheet material partially saturated with a water soluble stiffening agent and then saturated with thermo-plastic material.

11. A shoe stiffener comprising fibrous sheet material saturated through a portion of its thickness with a water soluble stiffening agent, and then saturated throughout with thermo-plastic material.

12. In the manufacture of shoe stiffeners the steps which comprise coating one face of fibrous sheet material with a water soluble stiffening agent, and then immersing the sheet in melted thermo-plastic material.

13. In the manufacture of shoe stiffeners, the steps which comprise coating one face of fibrous sheet material with glue, permitting the glue to dry, and then saturating the material and coating the glued face with thermo-plastic material.

14. In the manufacture of shoe stiffeners, the steps which comprise partially saturating fibrous sheet material with a stiffening agent softenable only when subjected to a solvent, permitting the material so treated to harden, and then further saturating the material with a stiffening agent softenable when subjected to heat.

15. In the manufacture of shoe stiffeners, the steps which comprise partially saturating fibrous sheet material with a stiffening agent in an aqueous vehicle, permitting the material to dry, and then further saturating the material with a thermoplastic.

16. A shoe stiffener comprising a layer of fabric impregnated with a waterproof thermoplastic stiffening substance and a superposed layer of fabric impregnated with a heat-resistant water-soluble stiffening substance.

In testimony whereof I have affixed my signature.

ALBERT L. CLAPP.

110

115

120

125

130